

March 3, 1936.

H. J. N. VOLTMANN

2,032,963

METHOD OF COLORING AND HARDENING STEEL

Filed Sept. 29, 1934



Inventor

Henry J. N. Voltmann,

By

Milburn & Milburn  
Attorneys

## UNITED STATES PATENT OFFICE

2,032,963

METHOD OF COLORING AND HARDENING  
STEEL

Henry J. N. Voltmann, Brooklyn, N. Y., assignor  
to W. S. Rockwell Company, New York, N. Y.,  
a corporation of New Jersey

Application September 29, 1934, Serial No. 746,232

3 Claims. (Cl. 148—16)

My invention relates to a method of coloring and hardening steel. The method is adapted to the treatment of steel and to imparting different colors to the metal. While it is particularly intended for use in the production of uniform razor blades with a uniform blue color, it is equally well adapted to the coloring and hardening of other products not only in strip or sheet form, but also in the form of tools, automotive parts and numerous other articles of steel. As is well known a blue color has been imparted to steel and especially to tool steel by drawing and tempering operations. The blued steel thus produced has not the requisite degree of hardness for the production of razor blades. In order to provide a sufficiently hard and otherwise satisfactory cutting edge the blade must be drawn back or tempered at a temperature (below 400° F.) relatively lower than that required for the production of blue oxide (between 500 to 600° F.).

The production of blued steel by annealing operations originally treated steel sheets in stacked relation, subjecting the sheets to an oxidizing agent at a comparatively high temperature and then lowering the temperature. The difficulty of uniformly heating or cooling steel while thus packed in a mass made it practically impossible to produce uniform razor blades of uniform color by such methods.

To obtain a product having the desired characteristics of hardness and uniformity of the cutting edge it has been found necessary to treat steel sheets or strips singly. The methods more recently employed, whether producing blued or plain blades, have involved the heating of the sheets or strips to a high temperature and rapidly chilling the heated steel. Where the blue color is not desired the heating is effected under customary furnace conditions. Where the blue color is to be produced on the hardened steel it has been proposed to carry out the heating to a high temperature (approximately 1400° F.) while the steel is enveloped in an oxidizing gas, the introduction of the gas for coloring and the application of the high temperature for hardening being performed simultaneously. By this method the gas employed for coloring the steel is introduced at a high temperature, at or above the critical or hardening point of the steel and considerably higher than the temperature required for the blueing operation.

In other words, the simultaneous coloring and heating for hardening have been performed at a temperature approximating that required for

hardening, and considerably higher than the temperature required and best suited for the blueing operation. At this temperature (approximately 1400° F.) the steel has a bright color.

The action of combustible gas at temperatures as high as 1400° F. or thereabouts is not clearly understood. Working with the gas at such temperatures is a delicate operation and is liable to give unexpected and unsatisfactory results. The composition of most gases is affected by such temperatures, so that the use of the different gases suitable for imparting a blue color or other color to the steel is made difficult and uncertain by the performance of the coloring operation in the high temperature hardening furnace and at the high hardening temperature. Different performance, more convenient operation and better results can be obtained by use of the gas or gases at a lower temperature.

My invention contemplates the production of a blued or colored sheet or strip by effecting the blueing or coloring with air or a suitable gas at a relatively low temperature (less than 1000° F.) and well below the critical temperature of the metal and the ignition point of the gas and subsequently heating the blued or colored metal to a higher temperature in a non-oxidizing atmosphere that does not affect the color established by the lower temperature.

The method which constitutes my invention consists in performing the coloring operation prior to and independently of the operation of heating for hardening.

The method further comprises the performance of the coloring operation at a relatively low temperature and a subsequent heating for hardening at a higher temperature.

The principal advantages of my method are better control of the finish; ease of varying the color of the metal by variation of the temperature or nature of the gas used for the coloring operation performed in a low temperature coloring zone out of the hardening zone and independently of the hardening operation; less danger of explosion; and elimination of odors or deposits from breakdown of the gas at the higher temperatures. By my method the coloring operation is performed under conditions best suited for effecting the desired results and does not in any way affect the proper hardening of the steel.

In practice my method is well adapted, but not limited, to the continuous coloring, hardening and tempering of a razor blade strip.

The coloring and subsequent heating opera-

tions may be performed in a single furnace by regulating the temperature within the furnace and the admission of the respective coloring and neutralizing gases to contact with the steel being treated. Or the successive operations may be effected in separate chambers or zones in a single furnace.

I have found it most practical and convenient to utilize separate chambers for the coloring operations and the subsequent high temperature heating for hardening, whether these chambers are separate furnaces or comprised in a single furnace. My invention does not reside in or depend upon the details of construction of the furnace or furnaces employed. By way of explaining the method and its operation and as an example of equipment which may be used, reference may be made to the apparatus illustrated diagrammatically in the accompanying drawing.

20 In this illustrative and preferred example of apparatus for carrying out my method the equipment comprises several units which may be individually distinct and separately mounted or may be combined and mounted upon a suitable stand adapted to be readily moved and handled as a single unit.

The several units or sections of the illustrated apparatus are a low temperature oxidizing or coloring furnace or chamber 1, a high temperature heating furnace or chamber 2 for hardening, a quench block 3 and a tempering unit 4. Suitable means (not shown) are also provided for pulling the razor blade strip 5 through the several units, chambers, sections or zones in succession, the strip being supported in any suitable manner for this purpose, for example, on a holding reel 6 and a take-off reel 7. The designation of the units as chambers is to be understood in its broad sense as referring to compartments, sections or zones of a single furnace as well as to separate furnaces.

The coloring chamber 1, hardening chamber 2 and tempering chamber 4 may be of any suitable construction, for example built with strong welded steel boxes lined throughout with insulating materials. The muffles 8, 9 and 10 respectively provided in these chambers or furnaces for the passage of the steel strip therethrough may be either single or double muffles constructed of nickel chromium heat-resisting alloy or of any other suitable material.

The chambers or furnaces 1, 2 and 4 may be electrically heated or gas fired. The strip 5, being heated within the muffles 8, 9 and 10 in either of these types of chambers does not come into contact with heating chamber gases. By this arrangement the operations of coloring and subsequent heating for hardening are carried out without interference and the same desired uniform quality and finish of the blades is obtained whether electric heating or gas firing is used in the chambers.

Provision is made for circulating air or introducing various other known oxidizing gases or liquids in the muffle 8 of the coloring chamber or section 1. Considerable variation in the color of the strip can be obtained by circulating the air in the muffle 8 at different temperatures following generally the lines of procedure in the ordinary tempering processes. Different colors can also be produced by selection of suitable oxidizing or coloring gases, the identity, characteristics and degrees of oxidation capabilities of which are well known in the art. In lieu of air or gas, either or both at different temperatures if desired, low temperature liquid baths, for example, nitre or

various suitable oils or chemicals, may be employed for immersion of the strip 5 in muffle 8 of the coloring chamber 1 as a basis for and means of producing the color. Any suitable means may be provided for introducing, regulating and controlling the supply of air, gas or liquid to the muffle 8 into contact with the strip 5.

In any event, regardless of the particular oxidizing or coloring medium used, the treatment of the strip 5 therewith is carried out and the color fixed at a relatively low temperature, at or above the required coloring temperature, but less than 1000° F.

The muffle 9 of the chamber, furnace section or furnace 2 is supplied, by any suitable valved or otherwise controllable supply means, with a proper regulated quantity of a neutral or non-oxidizing gas, for example, nitrogen or carbon dioxide, to provide a non-oxidizing atmosphere in the muffle 9 surrounding the strip 5 as it is drawn therethrough after having been colored in chamber 1.

The invention is not limited to or dependent upon the use of any specific gas in muffle 9, there being various gases, in addition to those mentioned, of well known characteristics which are suitable for this purpose; the choice of the particular gas is merely a matter of selection.

In the operation of my method the strip 5, after being blued or otherwise colored in the coloring unit, chamber, furnace or zone 1, is transferred to the zone, chamber or furnace 2 to be heated to a higher temperature for hardening. The strip, while in chamber 2, is heated to a temperature of approximately 1400° F., or at or above the critical or hardening point of the steel.

Following this high temperature heating the strip 5 is successively drawn through the quenching block 3 and tempering unit 4. The block 3 may be formed of opposed water-cooled ground and polished hardened steel plates, adapted to be opened by any suitable lever mechanism to insert the end of strip 5 at the beginning of the coloring and hardening operation and thereafter maintained in proper contact by tension springs 45 or other devices suitable for this purpose. Block 3 preferably abuts or is disposed adjacent to chamber 2.

Automatic temperature controlling pyrometers may be provided for regulating the temperatures in the separate furnaces or in the respective zones of a single furnace where the latter form of furnace construction and arrangement is used.

It is to be understood, however, that the regulating means for controlling and varying temperatures and the supply of gas or air to the muffles of the furnaces form no part of my invention, such means generally being old and well known in the art. The same is true of the chilling and tempering means and their details of construction. In other words, my invention is not concerned with the particular construction or arrangement of the apparatus employed in coloring and heating, or in the manner in which the steel strip or sheet is chilled and tempered after it has been heated for hardening, as, for example, in chamber or furnace 2, but consists essentially in my novel method of coloring steel in a suitable atmosphere substantially below the hardening temperature of the steel and subsequently hardening the colored steel by heating and chilling.

I claim:

1. The method of producing colored steel which comprises imparting color to the steel at a rela- 75

tively low temperature within the temperature range adapted to impart color to the steel and subsequently continuing the heating of the colored steel to a substantially higher temperature at or above the critical temperature of the steel being treated, and finally chilling the steel.

2. The method of coloring and hardening steel which comprises subjecting the steel to an oxidizing gas and while so subjected heating the steel to a temperature substantially below the critical point of the steel being treated and within the temperature range adapted to impart color to the steel; maintaining the steel in heated condition; subjecting the colored steel while still in heated condition to neutral gas; and heating the colored steel while subjected to the neutral

gas to a temperature at or above the critical point of the steel being treated.

3. The method of blueing and hardening steel which comprises introducing the steel into a coloring furnace and subjecting the steel in an oxidizing atmosphere therein to a relatively low temperature substantially below the critical point of the steel being treated and within the temperature range adapted to impart color to the steel; transferring the blued steel from the coloring furnace without intermediate cooling to a high temperature furnace, subjecting the blued steel therein to a temperature above the critical point of the particular steel being treated in contact with neutral gas, and then chilling the steel. 15

HENRY J. N. VOLTMANN.